

Patented Apr. 28, 1925.

1,535,858

# UNITED STATES PATENT OFFICE.

WILHELM ROHN, OF HANAU, GERMANY.

METAL AND METAL ALLOY FOR THERMOELECTRIC PURPOSES IN PARTICULAR FOR  
MAKING THERMOCOUPLES.

No Drawing.

Application filed May 14, 1920. Serial No. 381,520.

To all whom it may concern:

Be it known that I, Dr. WILHELM ROHN, chemist, a citizen of Germany, and resident of Hanau, Germany, have invented new and useful Metals and Metal Alloys for Thermo-electric Purposes in Particular for Making Thermocouples, of which the following is a specification.

For accurately measuring high temperatures, ranging from 600 to 1600° in practice and science chiefly the platinum-platinum-rhodium thermocouple after Le Chatelier is used. As long as they are protected against injurious influences, such as metal vapors, silicon, carbon etc., the wires made of these precious metals will bear the temperatures well and will not oxidize. Another great advantage of these couples is the possibility of exchanging them. Both metals, platinum and rhodium can be produced absolutely chemically pure and therefore will always display the same thermo-electrical properties. As both metals will remain unaffected in the air at their melting temperature; as they will neither evaporate and will not react on the crucible material, for producing the platinum-rhodium alloy, it is only necessary to weigh off the two components to the required exact weight and fuse them together without any special precautions. Provided the melt is kept liquid sufficiently long for the alloy become uniform, one may be certain to obtain alloys which will be thermo-electrically identical to all their predecessors and their successors. With the platinum, only chemically pure metal need be melted and drawn into wire. This affords the great advantage that the electric measuring instrument, the millivoltmeter, by means of which the thermo-forces are measured, need be gaged only once for the respective temperatures, to be certain, that all previously or subsequently made platinum-rhodium thermocouples, connected to this millivoltmeter, will always show the same temperature readings.

Notwithstanding these advantages the platinum-rhodium couple has certain disadvantages. The first is the comparatively low thermoforce, in consequence of which very sensitive measuring instruments are required to obtain a sufficiently ample and well readable stroke, and such measuring instruments are both expensive and easily sub-

ject to injury. A further drawback of the platinum-rhodium couples is their very high price. It is true, that when the couple is destroyed the platinum will remain a certain, very considerable value thereof, but frequently a good part of the metal is lost simultaneously with the destruction of the couple.

In view of these drawbacks, there has been for some time a tendency to replace the expensive platinum-rhodium thermocouples of small thermoforce, with thermocouples made of base metals, which may be used up to temperatures of 1200 or 1250° at least, which have a high thermoforce and are comparatively cheap. Base metals and alloys suitable for the purposes have been found and thermocouples made therefrom have been widely used. It was, however, impossible to convert base metals in chemically pure state, without impurities into the reguline form, and also to produce alloys of such base metals with such accuracy that charges of different provenience are sufficiently identical as regards their purity and composition and therefore also thermoelectrically. The reason for this lies in the fact that base metals, when melted in the presence of air, furnace gases and the like, will be partly oxidized, or partly burn away and will partly absorb impurities or react through their oxides with the material of the crucibles used. Furthermore alloys of such base metals will when melted in the manner customary in practice, undergo changes in their composition by the said circumstances acting differently on the various components of the alloy and also in each individual case. In consequence thereof it was not heretofore possible to produce in practice base metals and their alloys which were thermoelectrically identical, and each time a thermocouple was made of another melt, the measuring instruments had to be scaled afresh or suitable resistances had to be interposed between thermocouple and measuring instrument so as to reduce the stroke of the needle to the same degrees.

These drawbacks may be obviated if metals obtained pure by chemical means are electrically melted at a very low pressure or if alloys are thus made therefrom. It is thereby made impossible for them to absorb impurities or to oxidize; it is no more

necessary to employ reducing and purifying agents which might affect the thermoforce, and alloys cannot be subjected to changes by their components undergoing the injuries of the melting process to a various degree. My general process of melting metals is set forth in my co-pending application, Serial Number 363,916, filed March 6, 1920.

10 The vacuum melting process, therefore, permits the conversion of chemically pure metals into the reguline state without their purity and quality being impaired, and the production of metal alloys of such an accurate in composition that melts from different charges will be practically identical both as regards their physical properties and their chemical composition, and thus also thermoelectrically alike. By melting 20 in vacuo it is impossible for the metals to absorb impurities from the air or the furnace gases for them to burn away, or be oxidized and also for the oxides to react with the crucible material, so that the necessary accuracy is safeguarded. The vacuum melting process, furthermore allows remelting any amount of times metals and alloys without their absorbing impurities and without their changing their mechanical, physical and chemical properties. It is therefore possible to remelt an alloy, which after the first melt still shows small differences from the properties stipulated, once or even several times by adding small quantities of correcting additions and so obtain the required thermoelectric properties with the necessary accuracy. In short, by employing the vacuum melting process all those possibilities are opened to the full extent for thermocouples made of base metals which heretofore existed merely for such thermocouples made of precious metals or in particular of platinum-rhodium. The use of the vacuum melting process seems to afford also another advantage. By employing this process, which has been developed to the highest perfection, metals and alloys are obtained, which are free of even microscopical and submicroscopical gas inclusions and porosities. Therefore the atmospheric oxygen, to which the thermocouples are more or less exposed during use will not find any opportunity of attacking them, except on the surface of the wires.

55 In consequence thereof the destruction of such couples seems to proceed slower and to penetrate less deeply than with metals and

alloys obtained by the usual technical means.

Thermocouples made of wires of vacuum melted metals and alloys are in their thermoelectrical properties sufficiently identical from charge to charge, so that the measuring instruments need not be regaged afresh when it becomes necessary to exchange the couples. This renders unnecessary all makeshifts otherwise employed in such cases. It is no more necessary to keep a large reserve stock of thermocouples of the same melt, in order to avoid having to perform such regaging too frequently. It is no more necessary to keep wires from different melts separately in stock, and therefore mistakes with all their serious possible consequences are obviated.

The following is another proof of the importance of the improvement thereby obtained: It is possible to produce, so to say, artificial platinum-platinum-rhodium couples by utilizing certain ternary alloys, which, provided the proper composition, is maintained (indeed with an allowance limit of  $\frac{1}{100}\%$ ) will correspond within about 5 degrees with the platinum-rhodium thermocouples within the whole range from 600-1200° not only to the absolute reading but also in the form of the thermoforce curve. Whereas heretofore it was necessary to employ with multiple recording instruments platinum-rhodium couples only, even when part of the temperatures to be recorded by the said multiple instrument was below 1200° and thus would have admitted the use of base-metal thermocouples, it is now possible to use base metal thermocouples in combination with platinum-rhodium thermocouples, without any difference being noticed in the instruments of their records. This is a result which would not have been possible without the employment of the vacuum melting process.

What I claim is:

1. The method of preparing uniform base metals and base metal alloys for use in thermocouples, which comprises degasification by melting under predetermined reduced pressures and predetermined temperatures.
2. A thermocouple composed of practically degasified base metals or base metal alloys.

In testimony, that I claim the foregoing as my invention I have signed my name this 27 day of February 1920.

DR. WILHELM ROHN.